# EUROPEAN PATENT SPECIFICATION

(11) **EP 3 666 918 B1**
(45) Date of publication and mention of the grant of the patent: **23.02.2022**
(21) Application number: 19191488.6
(22) Date of filing: 13.08.2019
(51) Int. Cl.: C22C 38/06, C22C 38/18, C22C 38/28, C22C 38/14, C22C 38/04, C22C 38/02, C22C 38/00

(54) **FERRITIC STAINLESS STEEL EXCELLENT IN CORROSION RESISTANCE AND IMPACT RESISTANCE**
FERRITISCHER ROSTFREIER STAHL MIT HERVORRAGENDER KORROSIONSBESTÄNDIGKEIT UND SCHLAGZÄHIGKEIT
ACIER INOXYDABLE FERRITIQUE PRÉSENTANT UNE EXCELLENTE RÉSISTANCE À LA CORROSION ET AUX CHOCS

(30) Priority: 12.12.2018 KR 20180159642
(43) Date of publication of application: 17.06.2020
(73) Proprietor: HYUNDAI MOTOR COMPANY, Seoul 06797 (KR); Kia Corporation, Seocho-gu Seoul 06797 (KR)
(72) Inventor: KANG, Min Woo, 21387 Incheon (KR); LEE, Chung An, 18385 Gyeonggi-do (KR); HONG, Seung Hyun, 04422 Seoul (KR); KWON, Soon Woo, 15594 Gyeonggi-do (KR)
(74) Representative: Viering, Jentschura & Partner mbB Patent- und Rechtsanwälte

(56) References cited:
- EP-A1- 2 723 910
- EP-A1- 2 995 697
- EP-A1- 3 339 460
- DE-U1-202011 106 778

## Description

### TECHNICAL FIELD

The present invention relates to a ferritic stainless steel having improved impact resistance and corrosion resistance at high temperatures by suppressing formation of a sigma phase.

### BACKGROUND

Exhaust system components such as exhaust pipes, mufflers, and the like, of automobiles have been required to have thermal fatigue properties, high temperature fatigue properties and oxidation resistance. Generally, in the related art, ferritic stainless steel having high corrosion resistance by including chromium (Cr) as an alloy component has been mainly used for exhaust system components.

For instance, ferritic stainless steel for an exhaust system component contains 15 to 20% of chromium (Cr) to maintain corrosion resistance at high temperatures. In order to improve corrosion resistance, the content of an alloy element enhancing corrosion resistance such as chromium (Cr) or molybdenum (Mo) may be added, but, in this case, cost is increased due to an increase in the content of the high-priced alloy elements. In particular, a sigma phase may be formed, and as a fraction thereof may be increased, durability (impact resistance) may be deteriorated against expectations and corrosion resistance may also be deteriorated. Thus, in order to maintain excellent corrosion resistance and impact resistance, which are in a trade-off relationship with each other, at the same time, formation of the sigma phase include Fe, Si, Mn, Mo and Cr can be suppressed.

For instance, a conventional ferritic stainless steel may contain the sigma phase at a volume fraction of 5 to 20%. In this regard, a technique for reducing the volume fraction of the sigma phase in ferritic stainless steels has continuously been researched.

EP 2 723 910 A1 describes a heat-resistant Fe-Cr-Al alloy with low chromium vaporization rate comprising among others 1 to 4% tungsten and 0,25 to 2% niobium, wherein tungsten provides the high-temperature strength and creep strength.

EP 2 995 697 A1 discloses a stainless steel substrate for solar battery including among others 0,005 to 4% silicon, 0,05% phosphor or less and 0,01% sulfur or less, wherein the phosphor and the sulfur help in limiting an increase in the refining cost.

EP 3 339 460 A1 discloses a vibration-damping ferritic stainless steel material comprising among others from 0,01 to 0,6% nickel and from 0,1 to 1% silicon.

### SUMMARY

A ferritic stainless steel is provided having improved impact resistance and corrosion resistance at high temperatures so that the ferritic stainless steel may be used as an exhaust system component exposed to a high temperature environment. The ferritic stainless steel is obtained by suppressing formation of a sigma phase s.

The present invention provides a ferritic stainless steel with the features according to claim 1. Further preferred embodiments of the steel are described in the dependent claims.

Preferably, a volume fraction of a sigma phase formed in a temperature range of 300 to 900 °C may be less than 5 %.

The term "sigma phase" as used herein refers to a non-magnetic stage or phase mainly including iron and calcium in stainless steels, e.g., ferritic and austenitic stainless steels. For instance, the sigma phase may form at ferrite/austenite interfaces or boundaries and such intermolecular stage or phase may cause metal alloy or stainless steel to lose ductility, toughness, stability and corrosion resistance. In typical ferritic and austenitic stainless steels, precipitation of the sigma phase can be often observed in various series of stainless steels and can be precipitated under an elevated temperature environment, for example, casting, rolling, welding, forging, and aging. In certain embodiments, the sigma phase occurs during metallic exposure to a temperature range from 300 °C to 1000 °C, 300 to 900 °C, 400 to 900 °C or 500 to 900 °C.

Preferably, the volume fraction of the sigma phase formed in the temperature range of 300 to 900 °C may suitably be 0.5 % or less or may not be precipitated.

Preferably, the volume fraction of the sigma phase formed in the temperature range of 300 to 900 °C may not be precipitated.

Preferably, a volume fraction of Cr₃Si formed in the temperature range of 300 to 900 °C may suitably be 0.5% or less.

Preferably, a volume fraction of each of AlN and Al₂O₃ formed in the temperature range of 300 to 900 °C may suitably be 0.0001 % or less.

Preferably, a volume fraction of M₂₃C₆ formed in the temperature range of 300 to 900 °C may suitably be less than 0. 2%.

Preferably, a volume fraction of a laves phase formed in the temperature range of 300 to 900 °C may suitably be 0.2% or less.

Preferably, a pitting potential (Ept) of the stainless steel in 3.5 % of sodium chloride (NaCl) at a temperature of 25 °C may suitably be 300 mV_{SCE} or greater.

The term "pitting potential" as used herein refers to an electrochemical potential that corresponds to the least positive current and voltage at which pits develop or grow on a metallic surface and a corrosion pit initiates on a metallic surface. Typically, pitting for a stainless steel as used herein may be characterized electrochemically by the critical pitting potential (Ept). A time required for forming rust in a condition of 5 % of sodium chloride (NaCl) after 3 % of salt water is sprayed may be 250 days or greater.

Impact resistance strength of the ferritic stainless steel measured by a Charpy keyhole-notch impact test may suitably be 55 J or greater.

Further provided is an exhaust system component of a vehicle that includes the ferritic stainless steel as described herein.

Still further provided is a vehicle that include the exhaust system component as described herein.

### BRIEF DESCRIPTION OF THE DRAWINGS

FIG. 1 is a table showing exemplary steel compositions in Inventive Examples and Comparative Examples;
FIGS. 2 and 3 are tables showing various phases generated in Inventive Examples and Comparative Examples;
FIG. 4 is a table showing measured physical properties of exemplary stainless steel according to Inventive Examples and Comparative Examples;
FIG. 5 is a graph showing results of measuring corrosion amounts in Inventive Examples and Comparative Examples;
FIG. 6 is a graph showing results of calculating phase transformation for each temperature according to the content of aluminum (Al);
FIG. 7 is a graph showing results of calculating phase transformation for each temperature according to the content of nitrogen (N);
FIG. 8 is a graph showing results of calculating phase transformation for each temperature according to the total amount of zirconium (Zr), calcium (Ca), and magnesium (Mg); and
FIG. 9 is a graph showing results of calculating phase transformation for each temperature according to the content of carbon (C).

### DETAILED DESCRIPTION

Hereinafter, embodiments of the present invention will be described in detail with reference to the accompanying drawings. The present invention may be embodied in different forms and should not be construed as limited to the embodiments set forth herein. Rather, these embodiments are provided so that this invention will be thorough and complete, and will fully convey the scope of the present invention to those skilled in the art.

The terminology used herein is for the purpose of describing particular exemplary embodiments only and is not intended to be limiting of the invention. As used herein, the singular forms "a", "an" and "the" are intended to include the plural forms as well, unless the context clearly indicates otherwise. It will be further understood that the terms "comprises" and/or "comprising," when used in this specification, specify the presence of stated features, integers, steps, operations, elements, and/or components, but do not preclude the presence or addition of one or more other features, integers, steps, operations, elements, components, and/or groups thereof. As used herein, the term "and/or" includes any and all combinations of one or more of the associated listed items.

It is understood that the term "vehicle" or "vehicular" or other similar term as used herein is inclusive of motor vehicles in general such as passenger automobiles including sports utility vehicles (SUV), buses, trucks, various commercial vehicles, watercraft including a variety of boats and ships, aircraft, and the like, and includes hybrid vehicles, electric vehicles, plug-in hybrid electric vehicles, hydrogen-powered vehicles and other alternative fuel vehicles (e.g. fuels derived from resources other than petroleum). As referred to herein, a hybrid vehicle is a vehicle that has two or more sources of power, for example both gasoline-powered and electric-powered vehicles.

FIG. 1 shows various exemplary steel compositions in Inventive Examples and Comparative Examples, and FIG. 2 shows phases generated in Inventive Examples and Comparative Examples. Provided is a ferritic stainless steel that is optimized in the content of major alloy components to suppress formation of a structure or intermetallic phase (e.g., a sigma phase) that negatively affects physical properties of stainless steel. The ferritic stainless steel is disclosed in the appended claims.

Carbon (C) is contained in an amount of 0.015 wt% or less based on the total weight of the ferric stainless steel. Carbon (C) as used herein is an element effective for enhancing strength of stainless steel. For instance, Ti(C,N) may be formed to expect a precipitation strengthening effect and suppress high temperature structure growth (grain growth) such that an increased in creep strength and enhancement of tempering physical properties may be expected. However, when the content of carbon (C) is greater than 0.015 wt%, M₂₃C₆ carbide may be formed to deteriorate thermal impact characteristics.

Silicon (Si) is contained in an amount of 0.17 wt% or less based on the total weight of the ferric stainless steel. Silicon (Si) as used herein is an element that acts as a deoxidizer and increases oxidation resistance and castability. However, when the content of silicon (Si) is greater than 0.17%, a sigma phase may be formed to deteriorate impact resistance and corrosion resistance.

Manganese (Mn) is contained in an amount of 1.35 wt% or less based on the total weight of the ferric stainless steel. Manganese (Mn) as used herein improves hardenability and yield strength of steel. However, when the content of manganese (Mn) is greater than 1.35 wt%, a sigma phase may be formed to deteriorate impact resistance and corrosion resistance.

Chromium (Cr) is contained in an amount of 17 to 20 wt% based on the total weight of the ferric stainless steel. Chromium (Cr) as used herein is an important element to ensure corrosion resistance of stainless steel and to obtain solid solution strengthening effect and stabilize an austenite phase. However, when the content of chromium (Cr) is less than 17 wt%, oxidation resistance may be deteriorated, and when the content of chromium (Cr) is greater than 20 wt%, the austenite phase may be stabilized and a matrix structure may be changed to an austenitic system or duplex system.

Aluminum (Al) is contained in an amount of 3 to 5 wt% based on the total weight of the ferric stainless steel. Aluminum (Al), which is an element acting as a solubility enhancer, increases oxidation resistance and makes the structure finer and uniform. If the content of aluminum (Al) is less than 3%, a sigma phase may be formed to lower structure uniformity, and if the content of aluminum (Al) exceeds 5%, a negative phase such as Cr₃Si may be formed.

Titanium (Ti) is contained in an amount of 0.5 wt% or less based on the total weight of the ferric stainless steel. Titanium (Ti) as used herein forms carbides to improve precipitation strengthening and high temperature strength. When the content of titanium (Ti) is greater than 0.5%, a laves phase may be formed and impact resistance and corrosion resistance may be decreased. The content of titanium (Ti) is limited to a minimum value of 0.1 wt%. When the content of titanium (Ti) is less than 0.1 wt%, formation of AlN, which deteriorates strength and weldability at high temperatures, may be increased.

The content of nitrogen (N) is less than 0.02 wt% based on the total weight of the ferric stainless steel. Nitrogen (N) as used herein induces formation of carbonitride, for example, Ti(C,N) may be formed to obtain a precipitation strengthening effect and suppress high temperature structure growth (grain growth). As such, creep strength may be increased and tempering physical properties may be improved. However, when the content of nitrogen is greater than 0.02 wt%, formation of AlN is increased.

Oxygen (O) is contained in an amount of less than 0.001 wt% based on the total weight of the ferric stainless steel. Oxygen (O) forms inclusions to decrease impact resistance, and is controlled to be as low as possible. An upper limit value of oxygen (O) is 0.001 wt% in consideration of a removing process.

The sum of the contents of zirconium (Zr), calcium (Ca), and magnesium (Mg) is adjusted to 0.001 wt% to 0.01 wt% based on the total weight of the ferric stainless steel. Zirconium (Zr), calcium (Ca), and magnesium (Mg) as used herein serves as a deoxidizer. When the total content of zirconium (Zr), calcium (Ca), and magnesium (Mg) is less than 0.001 wt%, Al₂O₃ may be generated, and when the total content of Al₂O₃ is greater than 0.01 wt%, castability may be deteriorated.

Meanwhile, the remainder other than the above-mentioned components includes Fe and inevitably contained impurities.

In another aspect, in order to manufacture ferritic stainless steel having excellent corrosion resistance and impact resistance, molten steel having the composition described above may be continuously cast through a general method to produce a slab, the slab is re-heated, a post-treatment such as hot rolling, hot annealing, cold rolling, and cold annealing is subsequently performed thereon.

In one exemplary embodiment, by controlling the content of each component of the molten steel, formation of a phase, which negatively affects physical properties, is suppressed. For instance, a sigma phase is suppressed at a temperature of 300 to 900 °C, where an exhaust system component is typically used, by controlling the amount of Si, Mn, and Al which affects formation of a negative phase. The amount of Si, Mn, and Al satisfies [Equation 1] below. $\left(20Si+Mn\right) / Al < 0.7$

In [Equation 1], Si, Mn, and Al refer to the content (wt%) of each component.

Furthermore, the content of Zr, Ca, and Mg is further limited to suppress formation of AlN and Al₂O₃. The content of Zr, Ca, and Mg satifies [Equation 2] below. $0.001 \leq Zr + Ca + Mg \leq 0.01$

In [Equation 2], Zr, Ca and Mg refer to the content (wt%) of each component.

Hereinafter, exemplary embodiments of the present invention will be described using Inventive Examples and Comparative Examples.

An experiment was conducted to produce final products according to the production conditions of commercially produced ferritic stainless steel, and a hot plate obtained by hot rolling a slab continuously cast using a molten steel produced while varying the content of each component underwent hot annealing, cold rolling, and cold annealing as illustrated in FIG. 1.

For instance, as illustrated in FIG. 1, each slab continuously cast using molten steel adjusted in composition may be re-heated and hot-rolled in a temperature range of 1050 to 1100 °C and subsequently annealed at a continuous annealing line (CAL) for 90 seconds in a temperature range of 900 to 950°C. Thereafter, structures cold-rolled and cold-annealed samples were observed at a temperature of 300 to 900 °C, which is a temperature range at which an exhaust system component is generally used. Results thereof are illustrated in FIGS. 2 and 3.

As shown in the results illustrated in FIGS. 2 and 3, sample No. 18, which is Inventive Example satisfying the kind and content of the alloy components given in the present invention included Ti(C,N) and laves phase formed on the basis of ferrite as a matrix structure but a sigma phase was not formed. Although the laves phase, which negatively affects physical properties, was formed, a maximum volume fraction thereof was generated, for example, 0.13% of the laves phase was formed.

Meanwhile, in the case of samples No. 1 to No. 4, Comparative Examples which did not satisfy the kind or the content of the alloy components given in the present invention, Ti(C,N), sigma phase, laves phase, and G phase were formed on the basis of ferrite as a matrix structure. In particular, the sigma phase, which negatively affects the physical properties, was formed by 5% or greater based on a volume fraction and that the laves phase was formed by 0.2% or greater based on the volume fraction.

Further, samples No. 5 and No. 6, which are Comparative Examples, did not satisfy the condition of [Equation 1] and the sigma phase was formed by 17% and 18%, respectively.

In sample No. 7, which is Comparative Example exceeding the content of C given in the present invention, M₂₃C₆, a negative phase, was formed in by 0.2%. Here, M denotes metallic elements which are Fe, Cr, Mn, and Ti in the present invention.

Sample No. 8 is Comparative Example including the content of Si greater than the predetermined amount discussed above and the condition of [Equation 1] given in the present invention was not met, and Sample No. 9 is Comparative Example including the content of Mn greater than the predetermined amount discussed above in the present invention. In Sample Nos. 8 and 9, the sigma phase was formed by 10% and 8%, respectively.

Sample No. 10 satisfied most of the contents of the alloy elements given in the present invention, and the sigma phase and the laves phase, which are negative phases, were not formed. However, the content of Ti in Sampel No. 10 was less than the predetermined content of Ti as discussed above in the present invention. Since the content of Ti is less than a limit range, AlN, which deteriorates strength and weldability at high temperatures, was formed by 0.0002%.

Sample No. 11 is Comparative Example including the content of Ti greater than the predetermined amount as discussed above in the present invention such that laves phase was formed by 2.1%.

Samples No. 12 and No 13 are Comparative Examples that did not satisfy the content of Al given in the present invention. Sample No 12 contained the sigma phase formed by 7% when the content of Al was less than the predetermined range discussed above and sample No. 13 contained Cr₃Si formed by 0.8% as the content of Al is greater than the predetermined range discussed above.

Sample No. 14 is Comparative Example that did not satisfy the content of N given in the present invention. When the content of N is greater than the predetermined range discussed above, AlN was formed by 0.001%. Sample No. 15 is Comparative Example that did not satisfy the content of O given in the present invention, and when the content of O was greater than the predetermined range discussed above, Al₂O₃ was formed by 0.0002%.

Sample No. 16 is Comparative Example that did not satisfy the condition of [Equation 1] and the sigma phase was formed by 8%. Sample No. 17 is Comparative Example that did not satisfy the condition of [Equation 2] and the content of Zr, Ca and Mg was less than the condition of [Equation 2] so Al₂O₃ was formed by 0.0002%.

According to various exemplary embodiments, formation of Cr₃Si AlN, Al₂O₃, and M₂₃C₆, including the sigma phase and the laves phase, which are negative phases, are suppressed by controlling the kind and content of the alloy components to satisfy the conditions discussed above

Further, pitting potential, corrosion resistance, thermal expansion coefficient, and corrosion amount of the produced products were measured and evaluated, and results thereof are illustrated in FIGS. 4 and 5. As for pitting potential, a pitting potential of 3.5% of sodium chloride (NaCl) at a temperature of 25 °C was measured. The pitting potential was measured by a type of measurement instrument using saturated calomel electrode (SCE) as a reference point.

As for corrosion resistance, a time required for forming rust due to 5% of sodium chloride after 3% of salt water was sprayed.

Impact resistance was measured by a Charpy keyhole-notch impact test, and a corrosion amount was measured when exposed to the atmosphere at a temperature section of 600 to 900°C in which the exhaust system component is generally used.

As shown in FIG. 4, in the case of sample No. 18, which is Inventive Example satisfying the kind and content of the alloy components given in the present invention, the pitting potential (Ept) at 3.5% sodium chloride (NaCl) was measured as 300 mV_{SCE} at a temperature of 25°C. To the contrary, all of samples No. 1 to No. 4 were measured to be less than 300 mV_{SCE}. As the value of the pitting potential is higher, fitting resistance is excellent. Thus, the pitting potential was improved when the type and content of the alloy components of the present invention were satisfied.

Further, in the case of sample No. 18, which is Inventive Example satisfying the kind and content of the alloy components given in the present invention, a time required for forming rust due to 5% of sodium chloride (NaCl) after 3% of salt water was sprayed was measured to be 294 days, greater than 250 days compared to Comparative Examples No. 1 to No. 4 where rust was formed earlier than 250 days.

Further, in the case of sample No. 18, which is Inventive Example satisfying the kind and content of the alloy components given in the present invention, an impact resistance strength measurement value was measured as 62 J, and impact resistance strength measurement values of all of samples No. 1 to No. 4, which are Comparative Examples, were measured to be less than 55 J.

Further, in the case of sample No. 18, Inventive Example satisfying the kind and content of the alloy components given in the present invention, a coefficient of thermal expansion was measured as 11.5×10⁻⁶, however, coefficients of thermal expansion of samples No. 1 to No. 4, which are Comparative Examples, were measured as 12.3×10⁻⁶, 12.1×10⁻⁶,12.0×10⁻⁶, and 11.6×10⁻⁶, respectively.

As shown in FIG. 5, in the case of sample No. 18, which is Inventive Example satisfying the kind and content of the alloy components given in the present invention, the corrosion amount was remarkably reduced in the temperature range of 600 to 900°C, as compared with samples No. 1 to No. 4 of the Comparative Examples.

Further, in order to examine a phase formed according to a change in the content of Al at a temperature range of 300 to 900°C in which the exhaust system component is generally used, a phase formed in an alloy of 0.01C-0.1Si-0.1Mn-18Cr-0.2Ti-0.01N, while varying the content of Al, was examined, and results thereof are illustrated in FIG. 6.

As shown in FIG. 6, a precipitation temperature range of the sigma phase narrowed and the volume fraction decreased as the content of Al increased until the Al content reached 3%. In particular, when 3% of Al was added, stability of the sigma phase was significantly reduced so as not to be formed. Also, when the content of Al is greater than 5 wt%, Cr₃Si was produced.

Meanwhile, although Al is added by 3 wt% or greater, the sigma phase may be formed when the content of Si and Mn is large. In particular, the formation of the sigma phase may affect Si, Mn and Cr in this order in the alloy components, and the content of Si may have sensitivity of 20 times as compared with the content of Mn. As a result, the formation of the sigma phase was suppressed when the relational expression described in [Equation 1] was satisfied. This phenomenon is also confirmed with the results of samples No. 12 and 17.

In order to examine a region in which AlN is formed according to a change in the content of N, the region in which AlN was formed was examined, while varying the N content in the alloy of 0.01C-0.1Si-0.1Mn-4Al-18Cr-0.2Ti. Results thereof are shown in FIG. 7.

As shown in FIG. 7, AlN was formed when the content of N was 0.03 wt% or greater. Thus, the content of N is limited to be less than 0.02 wt%.

In order to examine a region in which Al₂O₃ is formed according to a total amount of Zr, Ca, and Mg, a region in which Al₂O₃ was formed was examined, while varying a total amount of Zr, Ca, and Mg in an alloy of 0.01C-0.1Si-0.1Mn-4Al-18Cr-02Ti-0.01N-0.00050. Results thereof are shown in FIG. 8.

As shown in FIG. 8, Al₂O₃ was formed when the total amount of Zr, Ca, and Mg was less than 0.001 wt% and that Al₂O₃ was not formed when the total amount of Zr, Ca, and Mg was greater than 0.01 wt%.

Further, in order to examine a region in which M₂₃C₆ is formed according to a change in the content of C, a region in which M₂₃C₆ was formed was examined, while varying the C content in an alloy of 18Cr-0.1Mn-0.1Si-0.2Ti-0.01N-4Al, and a phase transformation transition for each temperature as examined in a state in which the content of C was fixed to 0.02 wt%. Results thereof are shown in FIG. 9. As shown in FIG. 9, M₂₃C₆ was formed when the content of C is greater than 0.017 wt%, and M₂₃C₆ was formed by 0.2% when the content of C was 0.02 wt%. Therefore, it is advantageous that the content of C is 0.015 wt% or less to maintain the volume fraction of M₂₃C₆ at less than 0.2% to improve the physical properties of the stainless steel.

According to various exemplary embodiment of the present invention, the ferritic stainless steel has obtained excellent corrosion resistance and impact resistance at high temperatures at which the exhaust system component is generally used by suppressing formation of the sigma phase and by controlling the content of the alloy elements that affect formation of the sigma phase and the laves phase.

Further, the excellent corrosion resistance and impact resistance at high temperatures is maintained without adding high-priced alloy elements, and thus, cost are reduced as compared to other steel products that realize similar performance.

According to various exemplary embodiment of the present invention, the ferritic stainless steel may have obtained excellent corrosion resistance and impact resistance at high temperatures at which the exhaust system component is generally used by suppressing formation of the sigma phase and by controlling the content of the alloy elements that affect formation of the sigma phase and the laves phase.

Further, the excellent corrosion resistance and impact resistance at high temperatures may be maintained without adding high-priced alloy elements, and thus, cost may be reduced as compared to other steel products that realize similar performance.

## Claims

1. A ferritic stainless steel consisting of:
an amount of 0.015 wt% or less, excluding 0 wt%, of carbon (C),
an amount of 0.17 wt% or less, excluding 0 wt%, of silicon (Si),
an amount of 1.35 wt% or less, excluding 0 wt%, of manganese (Mn),
an amount of 17 to 20 wt% of chromium (Cr),
an amount of 0.1 to 0.5 wt% of titanium (Ti),
an amount of 3 to 5 wt% of aluminum (Al),
an amount less than 0.001 wt% of oxygen (O),
an amount of less than 0.02 wt% of nitrogen (N),
iron (Fe) constituting the remaining balance of the ferritic stainless steel,
all the wt% based on the total weight of the ferritic stainless steel,
wherein contents of Si, Mn, and Al satisfy [Equation 1], $\left(20Si+Mn\right) / Al < 0.7$
wherein Si, Mn, and Al in Equation 1 represent the content in wt% of each component,
wherein further comprising:
zirconium (Zr), calcium (Ca), and magnesium (Mg),
wherein contents of Zr, Ca and Mg satisfy [Equation 2] $0.001 \leq Zr + Ca + Mg \leq 0.01$
wherein Zr, Ca, and Mg in Equation 2 represent the content in wt% of each component.

2. The ferritic stainless steel of claim 1, wherein a volume fraction of a sigma phase formed in a temperature range of 300 to 900 °C is less than 5%.

3. The ferritic stainless steel of claim 2, wherein the volume fraction of the sigma phase formed in the temperature range of 300 to 900 °C is 0.5 % or less or is not precipitated.

4. The ferritic stainless steel of claim 3, wherein the volume fraction of the sigma phase formed in the temperature range of 300 to 900 °C is not precipitated.

5. The ferritic stainless steel of one of claims 1-4, wherein a volume fraction of Cr₃Si formed in the temperature range of 300 to 900 °C is 0.5 % or less.

6. The ferritic stainless steel of one of claims 1-5, wherein a volume fraction of each of AlN and Al₂O₃ formed in the temperature range of 300 to 900 °C is 0.0001 % or less.

7. The ferritic stainless steel of one of claims 1-6, wherein a volume fraction of M₂₃C₆ formed in the temperature range of 300 to 900 °C is less than 0. 2 %.

8. The ferritic stainless steel of one of claims 1-7, wherein a volume fraction of a laves phase formed in the temperature range of 300 to 900 °C is 0.2% or less.

9. The ferritic stainless steel of one of claims 1-8, wherein a pitting potential (Ept) of the ferritic stainless steel in 3.5 % of sodium chloride (NaCl) at a temperature of 25 °C is 300 mV_{SCE} or greater.

10. The ferritic stainless steel of one of claims 1-9, wherein a time required for forming rust in a condition of 5 % of sodium chloride (NaCl) after 3% of a salt water is sprayed is 250 days or greater.

11. The ferritic stainless steel of one of claims 1-10, wherein
impact resistance strength of the ferritic stainless steel measured by a Charpy keyhole-notch impact test is 55 J or greater.

## Patentansprüche

1. Ein ferritischer rostfreier Stahl, bestehend aus:
einer Menge von 0,015 Gew.-% oder weniger, ausgenommen 0 Gew.-%, Kohlenstoff (C),
einer Menge von 0,17 Gew.-% oder weniger, ausgenommen 0 Gew.-%, Silizium (Si),
einer Menge von 1,35 Gew.-% oder weniger, ausgenommen 0 Gew.-%, Mangan (Mn),
einer Menge von 17 bis 20 Gew.-% Chrom (Cr),
einer Menge von 0,1 bis 0,5 Gew.-% Titan (Ti),
einer Menge von 3 bis 5 Gew.-% Aluminium (Al),
einer Menge von weniger als 0,001 Gew.-% Sauerstoff (O),
einer Menge von weniger als 0,02 Gew.-% Stickstoff (N),
Eisen (Fe), das den Rest des ferritischen rostfreien Stahls ausmacht,
wobei alle Gew.-% auf das Gesamtgewicht des ferritischen rostfreien Stahls bezogen sind,
wobei die Mengen von Si, Mn und Al die [Gleichung 1] erfüllen,
(20Si+Mn)/Al < 0,7 [Gleichung 1]
wobei Si, Mn und Al in Gleichung 1 die Menge in Gew.-% einer jeden der Komponenten darstellen,
ferner aufweisend:
Zirkonium (Zr), Kalzium (Ca) und Magnesium (Mg),
wobei die Mengen von Zr, Ca und Mg die [Gleichung 2] erfüllen
0,001 ≤ Zr+Ca+Mg ≤ 0,01 [Gleichung 2]
wobei Zr, Ca und Mg in Gleichung 2 die Menge in Gew.-% einer jeden der Komponenten darstellen.

2. Der ferritische rostfreie Stahl gemäß Anspruch 1, wobei ein Volumenanteil einer in einem Temperaturbereich von 300 bis 900 °C gebildeten Sigma-Phase weniger als 5 % beträgt.

3. Der ferritische rostfreie Stahl gemäß Anspruch 2, wobei der Volumenanteil der im Temperaturbereich von 300 bis 900 °C gebildeten Sigma-Phase 0,5 % oder weniger beträgt oder nicht ausgeschieden ist.

4. Der ferritische rostfreie Stahl gemäß Anspruch 3, wobei der Volumenanteil der im Temperaturbereich von 300 bis 900 °C gebildeten Sigma-Phase nicht ausgeschieden ist.

5. Der ferritische rostfreie Stahl gemäß einem der Ansprüche 1 bis 4, wobei ein Volumenanteil des im Temperaturbereich von 300 bis 900 °C gebildeten Cr₃Si 0,5 % oder weniger beträgt.

6. Der ferritische rostfreie Stahl gemäß einem der Ansprüche 1 bis 5, wobei ein Volumenanteil von jedem von einem im Temperaturbereich von 300 bis 900 °C gebildeten AlN und Al₂O₃ 0,0001 % oder weniger beträgt.

7. Der ferritische rostfreie Stahl gemäß einem der Ansprüche 1 bis 6, wobei ein Volumenanteil des im Temperaturbereich von 300 bis 900 °C gebildeten M₂₃C₆ weniger als 0,2 % beträgt.

8. Der ferritische rostfreie Stahl gemäß einem der Ansprüche 1 bis 7, wobei ein Volumenanteil einer im Temperaturbereich von 300 bis 900 °C gebildeten Laves-Phase 0,2 % oder weniger beträgt.

9. Der ferritische rostfreie Stahl gemäß einem der Ansprüche 1-8, wobei ein Lochfraßpotential (Ept) des ferritischen rostfreien Stahls in 3,5 % Natriumchlorid (NaCl) bei einer Temperatur von 25 °C 300 mV_{SCE} oder mehr beträgt.

10. Der ferritische rostfreie Stahl gemäß einem der Ansprüche 1-9, wobei unter einer Bedingung von 5 % Natriumchlorid (NaCl) nach dem Besprühen mit 3 % Salzwasser eine Zeit, die für die Bildung von Rost erforderlich ist, 250 Tage oder mehr beträgt.

11. Der ferritische rostfreie Stahl gemäß einem der Ansprüche 1-10, wobei
eine Kerbzähigkeit des ferritischen rostfreien Stahls, gemessen im Charpy-Schlüsselloch-Kerbschlagbiegeversuch, 55 J oder mehr beträgt.

## Revendications

1. Acier inoxydable ferritique composé de :
une quantité de 0,015 % en poids ou moins, à l'exclusion de 0 % en poids, de carbone (C),
une quantité de 0,17 % en poids ou moins, à l'exclusion de 0 % en poids, de silicium (Si),
une quantité de 1,35 % en poids ou moins, à l'exclusion de 0 % en poids, de manganèse (Mn),
une quantité de 17 à 20 % en poids de chrome (Cr),
une quantité de 0,1 à 0,5 % en poids de titane (Ti),
une quantité de 3 à 5 % en poids d'aluminium (Al),
une quantité inférieure à 0,001 % en poids d'oxygène (O),
une quantité inférieure à 0,02 % en poids d'azote (N),
le fer (Fe) constituant le reste de l'acier inoxydable ferritique,
tous les pourcentages en poids sont basés sur le poids total de l'acier inoxydable ferritique,
dans lequel les teneurs en Si, Mn et Al satisfont à l'[Équation 1],
(20Si+Mn)/Al < 0,7 [Équation 1]
où Si, Mn et Al dans l'Équation 1 représentent la teneur en % en poids de chaque composant,
comprenant en outre :
du zirconium (Zr), du calcium (Ca) et du magnésium (Mg),
dans lequel les teneurs en Zr, Ca et Mg satisfont à [l'Équation 2] 0,001 ≤ Zr+Ca+Mg ≤ 0,01 [Équation 2]
dans lequel Zr, Ca et Mg dans l'Équation 2 représentent la teneur en % en poids de chaque composant.

2. Acier inoxydable ferritique selon la revendication 1, dans lequel une fraction volumique d'une phase sigma formée dans une plage de température de 300 à 900 °C est inférieure à 5 %.

3. Acier inoxydable ferritique selon la revendication 2, dans lequel la fraction volumique de la phase sigma formée dans la plage de température de 300 à 900 °C est de 0,5 % ou moins ou n'est pas précipitée.

4. Acier inoxydable ferritique selon la revendication 3, dans lequel la fraction volumique de la phase sigma formée dans la plage de température de 300 à 900 °C n'est pas précipitée.

5. Acier inoxydable ferritique selon l'une des revendications 1 à 4, dans lequel une fraction volumique de CrsSi formée dans la plage de température de 300 à 900 °C est de 0,5 % ou moins.

6. Acier inoxydable ferritique selon l'une des revendications 1 à 5, dans lequel une fraction volumique de chacun de AIN et Al₂O₃ formée dans la plage de température de 300 à 900 °C est de 0,0001 % ou moins.

7. Acier inoxydable ferritique selon l'une des revendications 1 à 6, dans lequel une fraction volumique de M₂₃C₆ formée dans la plage de température de 300 à 900 °C est inférieure à 0, 2 %.

8. Acier inoxydable ferritique selon l'une des revendications 1 à 7, dans lequel une fraction volumique d'une phase de laves formée dans la plage de température de 300 à 900 °C est de 0,2 % ou moins.

9. Acier inoxydable ferritique selon l'une des revendications 1 à 8, dans lequel un potentiel de piqûration (Ept) de l'acier inoxydable ferritique dans 3,5 % de chlorure de sodium (NaCl) à une température de 25 °C est de 300 mV_{SCE} ou supérieur.

10. Acier inoxydable ferritique selon l'une des revendications 1 à 9, dans lequel un temps nécessaire à la formation de rouille dans une condition de 5 % de chlorure de sodium (NaCl) après pulvérisation de 3 % d'eau salée est de 250 jours ou plus.

11. Acier inoxydable ferritique selon l'une des revendication1 à 10, dans lequel
la résistance aux chocs de l'acier inoxydable ferritique mesurée par un essai de choc de Charpy par entaille en trou de serrure est de 55 J ou plus.
